

Nov. 4, 1958

R. ANTONSEN

**2,859,106**

# PROCESS AND APPARATUS FOR REMOVING SULFUR FROM IRON

Original Filed Sept. 17, 1952



**Fig. 1**



**Fig. 3**



1

2,859,106

PROCESS AND APPARATUS FOR REMOVING  
SULFUR FROM IRON

Randolph Antonsen, Boston, Mass.

Original application September 17, 1952, Serial No. 310,069. Divided and this application September 15, 1955, Serial No. 534,447

3 Claims. (Cl. 75—59)

This invention comprises a new and improved process for removing sulfur from molten iron and simultaneously recovering the sulfur thus removed. It includes within its scope novel apparatus by which the process may be carried out.

The present application is a division of my copending application Ser. No. 310,069, filed September 17, 1952, now abandoned.

The established practice of reducing iron ore to metallic iron is to heat the ore in the presence of coke and lime in a blast furnace. Because both the ore and the coke usually contain large amounts of sulfur this element inevitably appears in the metal product. For many end uses the iron must be refined and this involves, among other things, the removal of sulfur. Were it not for the presence of sulfur many refining operations could be greatly shortened, notably in the open hearth manufacture of steel in which considerable time is required to work out the sulfur, and incidentally carbon which must be replaced.

I have discovered that a large proportion of the sulfur content of iron can be easily removed therefrom and recovered as a valuable by-product by continuously treating a portion of the slag while in the furnace and in contact with the surface of the molten iron to remove the available sulfur therefrom as by blowing an oxygen-containing gas therethrough thereby reducing the sulfur content of the main slag body. The sulfur combined with the oxygen as oxides of sulfur is then removed from the treating zone and separated and recovered in accordance with known methods.

The principle according to which the process of my invention proceeds is as follows. It has long been known that the basic constituents of slags produced in blast furnace operations possess an exceptional affinity for sulfur. Were it not for this fact, substantially all of the sulfur which is normally present in the raw materials of the process would combine chemically with the molten mass of iron during the refining process. In operation, however, as the molten metal and slag collect in the hearth of the furnace, the greatest percentage of the sulfur of the system is concentrated in the slag. The sulfur content of the slag is usually quite substantial; in fact, it has been recognized that slags from blast furnace operation could constitute an implementing source of sulfur for the production of sulfuric acid.

Of course, the extent to which slag removes sulfur from the system is dependent upon the concentration of the sulfur in the iron and in the slag, upon the equilibrium of the sulfur between the iron and the slag, and upon the amount of iron and slag present in the system at any given time. As sulfur is being continuously removed from the slag, mass equilibrium is never reached and sulfur will continuously transfer to the slag from the iron mass until a new equilibrium condition based upon the remaining relatively low sulfur contents of the two materials is approached and the furnace is tapped. Sulfur transfer takes place both from the molten pool of

2

iron on the hearth of the furnace and from the molten iron as it percolates through the slag.

An important feature of the process of my invention is that it is effective also for the removal of phosphorus from the molten iron. Since, during the slag-desulfurizing process, the slag tends to become more basic in nature it acquires a greater affinity for the compounds of phosphorus, as well as the compounds of sulfur. The elimination of phosphorus from the molten iron is, of course, very desirable and accompanies the removal of sulfur. Further, by maintaining a highly basic slag as this treatment does it will be possible to reduce the amount of limestone needed in the charge; thus making for savings in limestone and coke per ton of product, reducing the back pressure required on the blast and increasing capacity.

Accordingly, it is the principal object of this invention to provide a process for continuously removing sulfur from molten iron by reducing the sulfur content of the slag within the furnace while maintaining contact of the molten iron with the slag so reduced in sulfur content.

Another object of the invention is to produce iron in a continuous process having a low sulfur content by a process carried on entirely within the furnace and without requiring the addition of external heat.

These and other objects of this invention will be best appreciated and understood from the following description of an illustrative example of one way in which it may be advantageously put into practice taken in connection with the accompanying drawings in which,

Figure 1 is a view in vertical section of a blast furnace and auxiliary slag treater,

Figure 2 is an enlarged view, partly in elevation and partly in vertical section, of the slag treater, and

Figure 3 is a view in vertical section of the hearth portion of furnace equipped with integral peripheral treaters.

In the drawings is represented a typical blast furnace 10 provided with a stack section 12, a charging valve 14, a bosh 16, a gas withdrawal line 18 and a hearth or crucible section 24, having a metal tapping hole 26 for withdrawing molten pig iron and a slag tapping hole (cinder notch) 28 for withdrawing liquid slag, all in a known manner. The iron level is indicated by dashed line 20 and the slag level by dashed line 22. The furnace is of the usual construction, having a suitable refractory lining along the walls of the stack, the bosh and the hearth, and may be also provided with a suitable wall-cooling means (not shown) but well known in the industry.

Appurtenant to furnace 10 is a sulfur removing unit or treater 30. Upper and lower conduits 32 and 34 connect the treater 30 with the blast furnace 10, the lower conduit 32 being connected into the hearth section of the furnace above the normal level of the iron and below the normal top level of the slag. The upper conduit 34 is connected into the blast furnace above the normal top level of the slag. A trap 36 is provided in the upper conduit 34 to prevent blow back of gases from the furnace into the treater.

As shown in detail in Figure 2, the slag treater 30 consists of a metal shell 38 within which are a gas chamber 40, a bottom treating chamber 42 and a top chamber 44. Refractory floor 46 supported on piers 48 separates the gas and treating chambers 40 and 42 respectively and contains a plurality of orifices 50. Between chambers 42 and 44 is a refractory mass 52 supported on ring pier 54 through which pass a plurality of flues 56. These flues are preferably vertically aligned with orifices 50. A gas supply conduit 58 connects into gas

chamber 40 and a flue 60 is provided at the top of the treater.

In operation, when sufficient molten iron and slag have accumulated so that slag flows into conduit 32, oxygen or an oxygen-containing gas, preferably preheated, is introduced into gas chamber 40 through conduit 58 and flows upward through orifices 50, through the slag in chamber 42 and through flues 56. As soon as enough slag has accumulated in the treating chamber 42 it will be lifted by the gas stream through flues 56 into upper chamber 44. The slag thus lifted by the gas streams into the upper chamber flows back into the blast furnace through conduit 34. During its flow through the treater the slag is in contact with the oxygen in the lifting gas for a time sufficient to enable a substantial proportion of the sulfur in the slag to combine with the oxygen to form oxides of sulfur which percolate through and separate from the slag in the upper chamber and are withdrawn from treater 30 through gas flue 60.

So long as the reduction of iron ore is continued and slag and iron accumulate in the bottom of the blast furnace the circulation of slag to treater 30 is continued. The slag with greatly reduced sulfur content returning to the blast furnace through conduit 34 provides a slag having a composition reduced in sulfur, which as I have stated above, attracts the sulfur causing equilibrium of the slag and the pig iron to change and further causing a transfer of sulfur from the iron to the slag. The oxides of sulfur removed from treater 30 are recovered for further processing, for example, to produce sulfuric acid.

The apparatus shown in Figs. 1 and 2 is not claimed herein but forms the subject matter of my co-pending application, Ser. No. 659,727, filed May 16, 1957.

Various embodiments of apparatus in which the process of my invention may be carried out will readily be apparent to those skilled in the art. One such embodiment is illustrated in Figure 3. Instead of employing a separate treater as shown in Figure 2, a portion of the blast furnace itself is used as a treating chamber. This consists of an annular recess 62, or a plurality of recesses separated by radial partitions from one another, built into the side wall of the blast furnace. The recess is so constructed that it communicates with the furnace below the normal level of the slag pool and extends within the furnace wall above the top level of the slag thus providing a sealed marginal space above the surface of the slag therein separated from the main body of the slag by overhanging depending wall 63 while maintained in direct contact therewith.

Passing through the outer wall of the blast furnace 10 and into the bottom of the recess 62 and below the normal level of the slag pool is a plurality of gas ducts 64 through which oxygen or an oxygen-containing gas is introduced for the same purpose as when treater 30 is used. At the top of the recess is a plurality of gas outlet pipes 66 through which the oxides of sulfur and phosphorus are withdrawn.

In operation, when a sufficient marginal body of slag has accumulated to seal the recess 62 the flow of oxygen or other oxygen-containing gas is commenced. The

gas passes through the marginal body of slag within and below the recess and out vent pipes 66 carrying off the sulfur oxides formed in the process. As the sulfur content of the slag in the recess is reduced, there will be a withdrawal or migration of sulfur from the main slag body and a natural circulation of the slag will be set up due to the flow of gas through that portion of the slag in the recess. The sulfur content of the slag will continuously be reduced and sulfur will continuously enter the slag from the molten iron as described above.

It will readily be understood that the process of my invention is applicable to the refinement of metals by other means such as by the open hearth process. It is merely necessary that the metal from which sulfur, phosphorus and the like impurities are to be removed have a body of slag in contact with its surface.

Having thus disclosed my invention and described in detail an illustrative embodiment of it, I claim as new and desire to secure by Letters Patent:

1. A process for removing sulfur from the molten iron underlying a layer of slag in a blast furnace, which is characterized by the steps of forming a closed recess above a marginal portion of the slag layer in the furnace, forcing an oxygen-containing gas into the slag in said recess, and withdrawing sulfur oxides from the said recess while the slag therein remains merged with the slag layer in the furnace.

2. A process for removing sulfur from the molten iron underlying a layer of slag in a furnace, which is characterized by the steps of segregating a minor marginal portion of the liquid slag layer from the main body of the slag in the furnace, maintaining free liquid communication between the said two portions on all sides of the main body, and continuously treating the segregated portion with oxygen-containing gas to remove sulfur therefrom, thus causing a migration of sulfur into the segregated portion from the body portion of the slag layer.

3. A process for removing sulfur from molten iron underlying a layer of molten slag in a blast furnace, which is characterized by the steps of separating the layer of slag into a main inner body and a marginal body which surrounds and merges into the main body on all sides thereof, maintaining direct liquid communication and contact between the said bodies, and injecting oxygen-containing gas into the marginal body thereby removing sulfur therefrom, causing migration of sulfur outwardly from the main body of the slag layer into the marginal body and thus from the underlying iron into the main body of the slag.

#### References Cited in the file of this patent

#### UNITED STATES PATENTS

|           |        |       |               |
|-----------|--------|-------|---------------|
| 1,366,398 | Lund   | ----- | Jan. 25, 1921 |
| 1,415,183 | Lund   | ----- | May 9, 1922   |
| 1,443,920 | Levy   | ----- | Jan. 30, 1923 |
| 1,535,109 | Davies | ----- | Apr. 28, 1925 |
| 1,590,730 | Evans  | ----- | June 29, 1926 |
| 1,646,728 | Evans  | ----- | Oct. 28, 1927 |
| 1,753,891 | Jones  | ----- | Apr. 8, 1930  |